

## UNITED STATES PATENT OFFICE

TARIO KIKUTA, OF TOBATA, FUKUOKA KEN, JAPAN, ASSIGNOR TO TOBATA IMONO  
KABUSHIKI KAISHA, OF TOKYO, JAPAN, A CORPORATION OF JAPAN

METHOD OF MANUFACTURING STRONG BLACK HEART MALLEABLE CAST IRON

No Drawing. Application filed November 27, 1929, Serial No. 410,255, and in Japan September 10, 1929.

The present invention relates to a method of manufacturing strong black heart malleable cast iron, which consists in charging an annealing pot with white iron castings, 5 holding the same at a suitable temperature between 900° and 980° C. for twenty to fifty hours so as to graphitize the free cementite contained therein, then lowering the temperature down to a suitable temperature between 10 730° and 650° C. and holding the castings at that temperature for ten to fifty hours, thus not only graphitizing pearlitic cementite, but on the other hand by putting in iron oxide or other oxidizing agents of 15 4 to 15% by weight of the charge of the white iron castings in the pot, accomplishing de-carbonization of the white cast iron while it is held at a high temperature in parallel to the graphitization. The object 20 thereof is to obtain black heart malleable cast iron as strong as cast steel by carrying out the operation more economically and in shorter time than by the known method and at the same time by effecting the de-carbonization perfectly. 25

the longer time will be required for annealing. The principal object of employing packing material in such a method is to utilize the heat absorbed by it and cool slowly at a temperature range just below  $Ar_1$  50 transformation point, so that pearlitic cementite produced at  $Ar_1$  transformation point of iron after the graphitization of free cementite can be graphitized. The de-carbonization which takes place in using iron oxide packing in said known method and for reducing deformation of castings caused during the annealing due to the use of packing material is only a subsidiary action, and is not the main object of the annealing operation. This is the reason why sand or slag is employed more often than oxide in manufacturing black heart malleable cast iron. In the manufacture of white heart malleable cast iron, the de-carbonization being the 65 primary object, it is the well known fact that iron oxide is employed as packing material.

However, when packing material is used, it takes considerable time to heat the charge 70 of castings in the pot uniformly, because the packing material has big heat absorbing capacity in itself and further it is a poor conductor of heat. Consequently, it requires a larger quantity of fuel to anneal, increases 75 deterioration of the annealing pot and it has another disadvantage in that charging castings to or their discharging from the pot is naturally slow as compared with the method in which no packing material is used. 80

The annealing method in which white cast iron is graphitized in two stages without packing material is however accompanied by more or less decarbonization, but as the de-carbonization is effected mainly by oxygen 85 contained in the air present in the space inside the pot, its amount is very small. When black heart malleable cast iron is viewed from the metallographical point, temper carbon is distributed in globular form on the 90

This invention resembles the method of graphitizing in two stages the combined carbon contained in white cast iron without employing packing material as described in my 30 prior Patent No. 1,692,842, but differs in effecting the decarbonization by aid of iron oxide or other oxidizing agents put in the annealing pot amounting to from 4 to 15% of the charge of the castings as mentioned 35 above. According to the known annealing method using packing material, sand, iron oxide, slag, etc. are usually used as packing material and the space left in the annealing pot after it is charged with white iron castings is almost completely filled with such material so that when the castings have irregular or mechanical shapes as is quite often the case in malleable cast iron, the 40 quantity of these packing materials will become considerably large and consequently

ground of silico-ferrite and the tensile strength of black heart malleable cast iron is controlled by the quantity of this carbon. Therefore, if the content of this free carbon is reduced as much as possible, it is possible to product castings with high tensile strength such as steel. If, however, the carbon content in the melt of white cast iron is made smaller, the temperature ranges between liquidus and solidus lines, as will be seen from the iron-carbon diagram, will be extended and as a result increases liquid shrinkage, thus increasing the tendency of producing porous or rough parts in the interior of the casting and making it difficult to obtain sound castings. For this reason, it is preferable to restrict the carbon content in white cast iron to about 2.5%, and it is not advantageous from the foundry view point to make it below 2.2%. Therefore, the most advantageous method of obtaining strong and perfect black heart malleable cast iron is to maintain the carbon content of white cast iron at nearly 2.5% and make the subsequent annealing accompanied by the de-carbonization. However, for the purpose of effecting said de-carbonization, it is not advantageous to fill the annealing pot with such packing material as iron oxide, because it increases cost of annealing.

After careful research and many experiments, I have found that the object of the de-carbonization can be attained perfectly by adding to the charge in the pot 4 to 15% by weight of iron oxide, and I find it is preferable to effect the de-carbonization in this manner rather than by passing oxygen gas or air during the annealing operation through the castings, as the latter method produces an unfavorable result due to the excessive oxidation of the iron itself. It may be added that the oxidation of the iron can be almost prevented by employing the proper amount of a suitable oxidizing agent like iron oxide.

The following are examples of carrying this invention into practice by using two series of white cast iron having the following chemical constituents:—

|               | Carbon<br>(per cent) | Silicon<br>(per cent) | Manganese<br>(per cent) | Sulphur<br>(per cent) | Phosphorus<br>(per cent) |
|---------------|----------------------|-----------------------|-------------------------|-----------------------|--------------------------|
| 55 No. 1----- | 2.58                 | 1.16                  | 0.28                    | 0.057                 | 0.162                    |
| No. 2-----    | 2.60                 | 1.06                  | 0.25                    | 0.058                 | 0.164                    |

A small electric annealing furnace having a capacity of about 200 kilograms has been used.

#### EXAMPLE I

(With no de-carbonizing agent)

Amount of white iron castings charged (including test pieces), 108 kilograms.

Hours required for graphitization of the first stage, 29 at 925-980° C.

Hours required for graphitization of the second stage, 49 at 710° C.

The result of the annealing was good, 70 showing the following tensile strength and bending angle:—

| Number of sample material | Content of carbon (per cent) |                 |            | Tension test               |                             | Bending test |
|---------------------------|------------------------------|-----------------|------------|----------------------------|-----------------------------|--------------|
|                           | Before annealing             | After annealing | Difference | Tensile strength (kg./mm.) | Elongation in 2" (per cent) |              |
| No. 1-----                | 2.58                         | 2.52            | 0.06       | 33.62                      | 12.0                        | 150          |
| No. 2-----                | 2.60                         | 2.39            | 0.21       | 33.00                      | 13.0                        | 100          |

From this it will be seen that the amount of de-carbonization during the annealing is 85 only about 0.13% on an average.

#### EXAMPLE II

(With de-carbonizing agent) 90

Amount of white iron castings charged (including test pieces), 128 kilograms.

Graphitization of the first stage, 30 hours at 925-960° C.

Graphitization of the second stage, 49 95 hours at 710° C.

De-carbonizing agent, hematite (it was put in a vessel like a pan and placed at the bottom of the annealing pot), 6.4 kilograms (about 5%).

The result of annealing was satisfactory. The surface oxidization was hardly observed.

| Number of sample material | Content of carbon (per cent) |                 |            | Tension test               |                             | Bending test |
|---------------------------|------------------------------|-----------------|------------|----------------------------|-----------------------------|--------------|
|                           | Before annealing             | After annealing | Difference | Tensile strength (kg./mm.) | Elongation in 2" (per cent) |              |
| No. 1-----                | 2.58                         | 1.90            | 0.68       | 36.31                      | 17.0                        | 330          |
| No. 2-----                | 2.60                         | 1.98            | 0.62       | 37.01                      | 18.0                        | 360          |

The amount of de-carbonization is 0.65% on an average. The tensile strength and elongation are far greater than when no de-carbonizing agent was employed as in Example I. 115

#### EXAMPLE III

(With de-carbonizing agent) 120

Amount of white iron castings charged (including test pieces), 118 kilograms.

Hours for graphitization of the first stage, 24 at 925-980° C.

Hours for graphitization of the second stage, 49 at 710° C.

De-carbonizing agent, (same hematite for Example II was repeatedly used), 6.4 kilograms.

The annealing was satisfactory and the following results were obtained:—

| 5<br>Number of sample material | Content of carbon (per cent) |                 |            | Tension test               |                             | Bending test |
|--------------------------------|------------------------------|-----------------|------------|----------------------------|-----------------------------|--------------|
|                                | Before annealing             | After annealing | Difference | Tensile strength (kg./mm.) | Elongation in 2" (per cent) |              |
| 10<br>No. 1.....               | 2.58                         | 1.79            | 0.79       | 37.40                      | 16.0                        | Over 360     |
| No. 2.....                     | 2.60                         | 1.64            | 0.96       | 38.17                      | 16.0                        | Over 360     |

Thus, it will be seen that the average amount of de-carbonization is about 0.88% and the tensile strength and elongation are further improved. Hematite powder used as de-carbonizing agent has been reduced, and the amount of the reduced iron was 64%.

20 As regards these phenomena of decarbonization, I have measured each of them numerically and thus have not only made the mechanism of the de-carbonization clear, but also was able to determine the amount 25 of the de-carbonizing agent required to obtain the necessary amount of de-carbonization of castings. That is to say, the de-carbonization takes place chiefly owing to the catalytic action of carbon dioxide gas ( $\text{CO}_2$ ) 30 and the carbon contained in white cast iron is not only removed, but at the same time the oxygen contained in iron oxide is lost. Thus, the de-carbonization of white cast iron is accompanied by the reduction of iron oxide. 35 Therefore, the present method also serves to reduce iron sand.

I claim:

1. Method of manufacturing strong black heart malleable cast iron consisting in charging an annealing pot with white iron castings and with 4 to 15% by weight of iron oxide, maintaining the same at a temperature between 900° C. and 980° C. for a period of time varying from twenty to fifty hours so as to graphitize the free cementite contained therein, then lowering the temperature to between 730° C. and 650° C. and maintaining that temperature for a period of time varying from ten to fifty hours thus graphitizing pearlitic cementite and effecting de-carbonization of the white cast iron.

2. Method of manufacturing strong black heart malleable cast iron consisting in subjecting a charge of white iron castings together with iron oxide to the amount of 4 to 15% by weight of the white iron castings to a temperature between 900° C. and 980° C. for a period of time varying from twenty to fifty hours, then lowering the temperature to a point between 730° C. and 650° C. and maintaining that temperature for from a period of time varying ten to fifty hours.

In testimony whereof I have affixed my signature.

65 TARIO KIKUTA.